

# United States Patent

[11] 3,622,285

[72] Inventor **Charles E. Hayes**  
North Attleboro, Mass.  
[21] Appl. No. **883,262**  
[22] Filed **Dec. 8, 1969**  
[45] Patented **Nov. 23, 1971**  
[73] Assignee **Leach & Garner Company**

[54] **COMPOSITE WIRE OR THE LIKE**  
5 Claims, No Drawings

[52] U.S. Cl..... **29/199,**  
75/165  
[51] Int. Cl..... **B32b 15/02**  
[50] Field of Search..... **29/199;**  
75/165

[56] **References Cited**  
UNITED STATES PATENTS  
2,608,753 9/1952 Mooradian..... 29/199  
3,302,280 2/1967 La Plante ..... 29/199 X  
*Primary Examiner—L. Dewayne Rutledge*  
*Assistant Examiner—E. L. Weise*  
*Attorney—Barlow and Barlow*

**ABSTRACT:** An elongated article usually in the form of a wire having a core of beryllium copper which is completely surrounded in cross section or clad by an alloy containing a plurality of metals with gold having the greatest percentage and particularly adapted for electrical purposes. In some cases there may be a barrier between the core and the outer cladding to prevent migration between the cladding and the core.

## COMPOSITE WIRE OR THE LIKE

## BACKGROUND OF THE INVENTION

Heretofore there has been on the market materials known as L & G 226 and L & G 247 which have been platinum-containing alloys and thus relatively expensive materials. These two materials each have a normal composition as follows:

L & G 226  
 Palladium—35 percent  
 Platinum—10 percent  
 Gold—10 percent  
 Silver—30 percent  
 Copper—13.75 percent  
 Zinc—1.25 percent  
 L & G 247  
 Platinum—1.0 percent  
 Palladium—44.0 percent  
 Gold—0.5 percent  
 Silver—38.5 percent  
 Copper—13.6 percent  
 Nickel—1.0 percent  
 Zinc—1.4 percent

## SUMMARY OF THE INVENTION

The article comprises a core with a cladding embracing the

| Designation | Ni    | C    | Mn     | Fe     | S      | Si     | Cu     | Cr     | Al     | Ti     | Others                    |
|-------------|-------|------|--------|--------|--------|--------|--------|--------|--------|--------|---------------------------|
| Nickel 200  | 99.5  | 0.06 | 0.25   | 0.15   | 0.005  | 0.05   | 0.05   | —      | —      | —      | —                         |
| Nickel 201  | 99.5  | 0.01 | 0.20   | 0.15   | 0.005  | 0.05   | 0.05   | —      | —      | —      | 0.02 Mg 0.04              |
| Nickel 205  | 99.5  | 0.06 | 0.20   | 0.10   | 0.005  | 0.05   | 0.05   | —      | —      | —      | 0.02 Mg 0.04              |
| Nickel 220  | 99.5  | 0.06 | 0.12   | 0.05   | 0.005  | 0.03   | 0.03   | —      | —      | —      | 0.003 Mg 0.06             |
| Nickel 230  | 99.5  | 0.09 | 0.10   | 0.05   | 0.005  | 0.03   | 0.01   | —      | —      | —      | 0.003 Mg 0.07             |
| Nickel 233  | 99.5  | 0.09 | 0.18   | 0.05   | 0.005  | 0.03   | 0.03   | —      | —      | —      | —                         |
| Nickel 270  | 99.98 | 0.01 | <0.001 | <0.001 | <0.001 | <0.001 | <0.001 | <0.001 | <0.001 | <0.001 | {Co <0.001<br>(Mg <0.001) |

core. A beryllium copper core has excellent spring characteristics, high-bulk electrical conductivity and excellent formability, and is a low-density material for reduced contact bounce while the covering or cladding over the core can be heat-treated in the same temperature range as the core, with excellent corrosion resistance on the contact surface, excellent contact wear and is suitable for welding, brazing or soldering with a substantial cost saving of up to 50 percent over the material set forth in the Background of the Invention. A barrier of nickel may be placed between the core and its cladding. The composite is highly satisfactory and in many cases exhibits superior performance for contact arms, buss bars, wiper blades and make and break applications in relays.

## DESCRIPTION OF THE PREFERRED EMBODIMENT

The article comprises an elongated form, such as wire, having a core and a cladding or coating about the core with often a barrier between the two.

The core is beryllium copper which contains percentagewise by weight 1.80–2.05 beryllium; 0.20 to 0.60 nickel or cobalt or some of each and the balance to 100 percent of copper. This composition is chosen for the spring characteristics and the electrical conductivity and also for low-density material for reduced contact bounce and ease of formability.

The cladding or coating completely encircles the core in cross section and is an alloy containing the following composition percentages by weight:

gold—40 to 60  
 palladium—9.6 to 14.4  
 silver—4.8 to 7.2  
 copper—19.2 to 28.80  
 nickel—4.8 to 7.2  
 zinc—1.6 2.4

This cladding alloy is chosen for its excellent corrosion resistance on a contact surface, its excellent contact wear, the fact that it is suitable for welding, brazing or soldering together with the fact that it has the same temperature range 75

as the beryllium copper of the core so that the two may be advantageously heat-treated together. There is also present a cost saving of up to 50 percent over the materials mentioned in the Background of the Invention because of the reduction or absence of some of the precious metals, such as platinum, from the claddings mentioned in the Background of the Invention.

A 10 percent by weight cladding has been found satisfactory although this percentage may be widely varied.

10 Although there is a range of the materials in the claddings mentioned above, a composition which has been found exceptionally good and within the range above mentioned is the percentage as follows:

gold—56.25  
 copper—21.00  
 palladium—10.50  
 silver—5.25  
 nickel—5.25  
 zinc—1.75

20 In some cases it is found that there may be a migration of the cladding material into the core or vice versa, and in order to prevent this migration a barrier may be placed between the core and the cladding which will be essentially nickel in a percentage by weight of 99 percent or over. The following cladding alloys may be used are denoted on the market as Huntington alloys and having the compositions as set forth in the following table;

25 Nickel 200  
 Nickel 201  
 Nickel 205  
 Nickel 220  
 Nickel 230  
 Nickel 233  
 Nickel 270

In the cladding material above specified where the end use is to have considerable wear, the amount of gold in the cladding composition may be increased to withstand such wear. Normally the gold alloy will be used in amounts ranging from 5 to 15 weight percent of the composite.

30 The above composite material for the cladding will serve as a low-cost substitute for solid gold or platinum, silver, palladium alloys, or the alloys specified in the Background of the Invention and still will offer equal or superior physical, chemical, or electrical properties. They have high reliability for spring contacts, primarily because of the following properties: they are highly tarnish and corrosion resistant; they have good spring properties with a Young's modulus of 16.5 to  $18 \times 10^6$  and yield strengths in the range of 140,000 to 180,000 p.s.i.; they have high hardness in the range of 350 to 420 D.P.H. which combined with the lubricity of the precious metals results in excellent wear characteristics; and they are age hardenable.

35 Some typical properties exhibited of the composite wire having a cladding of 10 weight percent and wire referred to in the Background of Invention are:

| Material  | Condition | Young's Modulus | Ultimate tensile strength (p.s.i.) | Elongation (percent) |
|-----------|-----------|-----------------|------------------------------------|----------------------|
| Invention | A         | —               | 79,000                             | 45                   |
| 226       | A         | —               | 105,000–135,000                    | 25–35                |
| 247       | A         | —               | 90,000–130,000                     | 30                   |
| Invention | AT        | 18.0            | 191,000                            | 1                    |
| 226       | AT        | 17.0            | 175,000–200,000                    | 5–10                 |
| 247       | AT        | 16.0            | 165,000–215,000                    | 2–12                 |
| Invention | 1/2 HT    | 18.0            | 200,000                            | 1                    |
| Do        | A         | —               | 79,000                             | 45                   |
| Do        | 1/2 H     | —               | 113,000                            | 4                    |
| Do        | 1/2 H     | —               | 127,500                            | 2–3                  |
| Do        | 1/2 II    | —               | 139,000                            | 1                    |
| Do        | II        | —               | 152,000                            | 1                    |
| Do        | AT        | 18.0            | 191,000                            | —                    |
| Do        | 1/2 HT    | 18.0            | 104,000                            | —                    |
| Do        | 1/2 HT    | 18.0            | 189,500                            | —                    |
| Do        | 1/2 IIIT  | 18.0            | 201,000                            | —                    |
| Do        | HT        | 18.0            | 207,000                            | —                    |

In the above table, the letter A represents the solution annealed condition: The letter H, which may be preceded by a number, represents a degree of work hardening; and the letter T following either A or H indicates that an age-hardening treatment has been given to the material. These designations are common metallurgical terms.

The above comparison shows certain superiorities of the cladding on the beryllium copper here set forth.

I claim:

1. A clad metal for electrical applications comprising a metal alloy core containing predominantly copper with from 1-3 percent by weight beryllium, said core in cross section being completely encircled with a cladding having the following composition percent by weight

Gold—40-60.

Palladium—9.6-14.4

Silver—4.8-7.2

Copper—19.2-28.80

Nickel—4.8-7.2

Zinc—1.6-2.4

2. A clad metal as in claim 1 wherein the core contains

|              |                        |
|--------------|------------------------|
| beryllium    | 1.80-2.05              |
| nickel or    |                        |
| cobalt or    |                        |
| some of each | 0.20-0.60              |
| copper       | balance to 100 percent |

3. A clad metal as in claim 1 wherein the cladding material is

|    |                 |
|----|-----------------|
| 10 | gold—56.25      |
|    | palladium—10.50 |
|    | silver—5.25     |
|    | copper—21.      |
|    | nickel—5.25     |
| 15 | zinc—1.75       |

4. A clad metal as in claim 1 wherein there is a barrier metal between the core and cladding, the barrier material having nickel in a percentage by weight of over 99 percent.

5. A clad metal as in claim 1 wherein the barrier metal is 20 99.5 percent nickel.

\* \* \* \* \*

25

30

35

40

45

50

55

60

65

70

75